# EUROPEAN PATENT APPLICATION

(11) **EP 0 459 474 A1**
(43) Date of publication of application: **04.12.1991**
(21) Application number: 91108843.3
(22) Date of filing: 29.05.1991
(51) Int. Cl.: C22C 26/00

(54) **Diamond-containing materials and a method of making products from the same**

(30) Priority: 01.06.1990 US 532478
(71) Applicant: UNITED TECHNOLOGIES CORPORATION, Hartford, CT 06101 (US)
(72) Inventor: Bluege, John, Lake Park, Florida 33403 (US)
(74) Representative: Klunker . Schmitt-Nilson . Hirsch

(57) **Abstract**

A composite material includes a multitude of diamond particles that are embedded in and interconnected by a matrix of a metallic material to form a solid body having a very high stiffness to weight ratio. A product having a very high stiffness to weight ratio is made by mixing diamond particles with a particulate metallic material to obtain a mixture having a predetermined ratio of the diamond particles to the metallic material. A quantity of this mixture is then confined in an enclosed space which is then evacuated. Thereafter, the quantity of the mixture confined in the evacuated enclosed space is subjected to temperature and pressure conditions sufficient to cause the metallic material to form a matrix embedding and interconnecting the diamond particles to form a solid body therewith.

## Description

### Technical Field

The present invention relates to composite materials in general, and more particularly to lightweight composite materials with very high stiffness, and to a method of making products from such materials.

### Background Art

There are already known various lightweight high-strength materials that are being used for making products or structures, among them so-called composites that are constituted by intimate mixtures or agglomerations of two or more generally disparate materials that are bonded together by other than chemical bonds and each of which contributes its inherent properties to the composite so that the overall properties of the composite material are superior to those of either of the constituent materials if it were used by itself. The material to be used for a particular product, component or structure, be it a single element material or a composite material, is usually chosen in such a manner as to give the respective product, component or structure the attributes or properties required or expected therefrom, such as the required strength, resistance to wear, chemical attack or other external influences to which the component, product or structure is subjected or exposed when in use, and the like.

In most terrestrial applications, the cost of the materials going into the product, and the cost of manufacturing the product, are also important if not determinative factors in selecting the materials. However, in certain other applications, such as in the aeronautical, astronautical and deep sea fields, such costs may become only secondary factors that may be outweighed by other considerations, such as the cost of bringing the product into outer space or of repeated lifting of the product when the platform carrying the same becomes airborne. Especially in these applications, it is desirable if not imperative to keep the weight of the product to the minimum, obviously without sacrificing the desirable properties of such product.

Thus, for instance, high performance mirrors and structures must perform in a stable and reliable manner under severe thermal and/or environmental conditions which necessitate high thermal conductivity, low thermal expansion, high stiffness, and radiation hardness. Applications include mirrors for high energy lasers and orbital surveillance as well as aerospace and other structures requiring very high stability and/or specific stiffness (aircraft, satellites, etc.). Currently, the preferred materials of choice for such products are molybdenum, silicon, and silicon carbide for the laser mirrors and beryllium and silicon carbide for the aerospace applications.

Diamond offers dramatic performance improvements over all of these materials. In particular, its unexcelled specific stiffness would make it desirable to use it in the construction of thermo-mechanically stable structures of the lowest possible weight. However, it was heretofore impossible to employ diamond as a structural material, except in some rare instances, not only because of cost concerns, but also, and probably more importantly, because there is no currently known method of synthetically producing pure diamond products of any meaningful size that would be required for such products to be employable in the above applications.

In view of the above, beryllium, which has the highest specific stiffness of all of the materials that are currently considered to be available for the making of products of the above type, is often resorted to for making such products. Unfortunately, beryllium is also costly (albeit less so than pure diamond), and it also poses a fabrication health risk, and requires high fabrication temperatures (about 1200^{o}C). Moreover, inasmuch as beryllium tends to crystallize in an anisotropic fashion, products such as structures, structural components, mirrors or the like that are made of this material exhibit thermal, temporal and polishing instabilities which would not be present if such products were made of or with diamond because the latter forms isotropic crystals.

Accordingly, it is a general object of the present invention to avoid the disadvantages of the prior art.

More particularly, it is an object of the present invention to provide a material for use in lightweight, high-strength products, which material does not possess the disadvantages of the known materials currently used for making products of this kind.

Still another object of the present invention is so to develop the material of the type here under consideration as to be suited for use in the production of a wide variety of products regardless of their sizes and/or shapes.

It is yet another object of the present invention to devise a method of making products from the material of the above type, which method would render it possible to give the respective product any desired size and shape.

A concomitant object of the present invention is to design an equipment for the performance of the method of the above type in such a manner as to be relatively simple in construction, inexpensive to manufacture, easy to use, and yet reliable in operation.

### Disclosure of the Invention

In keeping with these objects and others which will become apparent hereafter, one feature of the present invention resides in a composite material which includes a multitude of diamond particles and a matrix of a metallic material embedding the diamond particles and interconnecting the same to form therewith a solid body having a very high stiffness to weight ratio.

According to another aspect of the present invention, there is provided a method of making a product having a very high stiffness to weight ratio, this method including the steps of mixing diamond particles with a particulate metallic material to obtain a mixture thereof with a predetermined ratio of the diamond particles to the metallic material; confining a quantity of the mixture in an enclosed space; evacuating the enclosed space; and subjecting the quantity of the mixture confined in the evacuated enclosed space to temperature and pressure conditions sufficient to cause the metallic material to form a matrix that embeds and interconnects the diamond particles to form a solid body therewith.

### Best Mode for Carrying Out the Invention

In accordance with the present invention, there is provided a composite material constituted by a solid mixture of diamond particles embedded in a matrix constituted by any of a variety of suitable matrix materials, preferably metals or metal alloys. Diamond can be mixed with many materials, including metals, with no reaction, because it is among the most chemically inert of all known materials. This property allows the formation of mixtures of diamond and other materials to form composites with very well defined constituent ratios. Mixtures are known to follow classical mixture rules which predict that properties such as expansivity, conductivity and the modulus of elasticity vary smoothly, albeit not necessarily linearly, with relative constituent ratios. When metals are used as the matrix materials, they form a high thermal and electrical conductivity matrix that embeds and positionally fixes the inert diamond particles. Additional materials can also be used in the mixture, and they can later be leached out to form a porous structure suitable for very high performance heat exchangers (with well defined porosity) as well as for catalytic and ion exchange structures suitable for use in environments otherwise unsuitable for organic media.

The composite materials described here make it possible to achieve very high performance close to that of pure diamond in a manner that is cost effective and scalable. A solid mixture of diamond powder and particles of one or more low density metals forms a family of solids with unexcelled stiffness, high thermal and electrical conductivity, low thermal expansivity and relatively low fabrication temperatures, and enables the use of such solids in structural/thermo-mechanical applications that are not achievable using other materials.

In accordance with another aspect of this invention, the diamond composite is formed by mixing diamond and metal powders, sealing the mixture in an evacuated mold or other evacuated space, and subjecting the mixture to high temperature and pressure until the metal has infiltrated the interstices between the diamond particles. Then, upon cooling of the thus treated composite material, the metallic material will embed and interconnect the diamond particles, resulting in the formation of a solid body. When the evacuated space is constituted by a mold cavity, it is possible, by appropriately selecting the shape of the mold cavity and/or any mandrels contained in or projecting into this cavity, and/or the means that exerts the required pressure on the quantity of the mixture that is confined in the mold cavity, to give the thus obtained solid body a shape that is very close to, if not identical with, that of the final product. Under these circumstances, only a minimum amount of, if any, machining, such as grinding or polishing, is required to give the solid body is final configuration, appearance and/or surface texture or quality.

As already mentioned before, there is a wide range of materials, such as metals and metal mixtures, that can be used for the matrix. As an example, composites of the above type using magnesium or aluminum (convenient low density metals) for the matrix material can typically be formed or shaped at 550^{o}C (versus 1200^{o}C needed for forming products from beryllium) and 15000 psi, although lower pressures can be used. While experience indicates that the above temperature and pressure parameters are suitable when either aluminum or magnesium is employed as the matrix material, the actual choice of such parameters depends on which metal is selected to constitute the matrix, on the complexity of the shape of the product to be made, and on other criteria. The only substantive limitations on the temperature range are the temperature at which the metal is capable of flowing at the pressure applied into the interstices between the diamond particles (generally speaking, the plastic deformation point) at the lower end, and the graphitization of the carbonaceous material of the diamond particles at the upper end. Thus, the preferred temperature range for aluminum or magnesium is between 500 and 1200^{o}C. The diamond volume fraction in the mixture is typically chosen to be as high as in the 80-95 percent range to assure bonding, on the one hand, and properties as close to those of pure diamond as possible or feasible.

Mixtures that are comprised of nonalloying or nonreactive species are remarkably predictable by simple mixture rules. The properties tend to vary quite monotonically between those of the constituents. Thus, composite materials having the aforementioned high ratio of diamond particles to the matrix material will exhibit stiffness that is very close to that of pure diamond.

The major properties of interest to the high performance mirror industry are listed in the accompanying Table 1. Values are included for the materials mentioned above as well as for diamond.

As indicated above, diamond offers dramatic improvement in component weight and thermal stability relative to other materials heretofore used for making products for similar applications. Since, as mentioned before, diamond cannot yet be fabricated in large sizes, composites offer the means to achieve most of the advantages of pure diamond, but at a cost competitive with other high performance structure materials.

The use of low density metals such as aluminum or magnesium allow the fabrication of diamond-metal composites at about half the temperature required to form beryllium and with improved isotropy. Thus, diamond-metal composites offer higher performance, lower fabrication temperatures, improved thermal and mechanical performance, lower susceptibility to thermal and temporal instabilities and no toxicity when compared to beryllium and silicon carbide which are currently considered the best materials available.

The improved material properties provide enhancements in performance and stability, and/or a reduction in weight. For example, the fact that the specific stiffness of diamond is double that of its closest competitor, beryllium, enables the use of a lighter design which, in turn, eases the launch requirements and/or allows the use of a larger, more efficient collection aperture for orbital surveillance satellites.

Or, as another example, if the weight of a satellite is equally divided between structure (made of beryllium) and payload, the use of a diamond composite instead of beryllium would increase the payload capacity by up to 50 percent for the same total launch load. Since diamond powder costs are relatively low (about the same in terms of dollars per pound as those of zinc selenide), such composites can be used for high performance airframes, such as the national aerospace plane and hypersonic missiles, with comparable gains in payload and performance. In fact, the higher performing diamond composite would enable applications which are well beyond the capabilities of current materials and designs.

Where cooling is required, the higher ratio of thermal conductivity to expansivity of diamond as compared with those of the other materials included in Table 1 allows the use of very high performance heat exchanger designs not available to any other material. Such devices are useful not only for cooled mirrors, but for high flux nuclear reactors, as well.

Thus, it may be seen that the material of the present invention, and the products made therefrom by using the method of the present invention, have the following advantages relative to the conventional ones:
- Very high specific stiffness (comparable to or higher than beryllium, unlike silicon carbide)
- Very high thermal conductivity (can be higher than that of copper)
- Very low thermal expansivity
- Excellent radiation hardness
- Nontoxic
- Can be formed to near final shape
- Property uniformity (isotropic unlike beryllium)
- Low temperature fabrication (half that of beryllium)

While the present invention has been described above as embodied in composites of a particular composition, it will be appreciated that the present invention is not limited to this particular example; rather, the scope of protection of the present invention is to be determined solely from the attached claims.

## Claims

1. A composite material comprising
a multitude of diamond particles; and
a matrix of a metallic material embedding said diamond particles and interconnecting the same to form therewith a solid body having a very high stiffness to weight ratio.

2. The composite material as defined in claim 1, wherein said metallic material of said matrix is aluminum.

3. The composite material as defined in claim 1, wherein said metallic material of said matrix is magnesium.

4. The composite material as defined in any one of claims 1 to 3, wherein the ratio of said diamond particles contained in said body to the metallic material is substantially in the range between 80 and 95%.

5. A method of making a product having a very high stiffness to weight ratio, comprising the steps of
mixing diamond particles with a particulate metallic material to obtain a mixture thereof with a predetermined ratio of the diamond particles to the metallic material;
confining a quantity of the mixture in an enclosed space;
evacuating the enclosed space; and
subjecting the quantity of the mixture confined in the evacuated enclosed space to temperature and pressure conditions sufficient to cause the metallic material to form a matrix embedding and interconnecting the diamond particles to form a solid body therewith.

6. The method as defined in claim 5, wherein the metallic material is aluminum.

7. The method as defined in claim 5, wherein the metallic material is magnesium.

8. The method as defined in any one of claims 5 to 7, wherein said confining and subjecting steps are performed in such a manner that the shape of the solid body at least substantially corresponds to that of the final product at the conclusion of said subjecting step.

9. The method as defined in any one of claims 5 to 8, wherein the conditions prevailing during said subjecting step are a temperature in the range of between about 500 and 1200^{o}C and a pressure of about 15000 psi.

10. The method as defined in any one of claims 5 to 9, wherein the predetermined ratio is substantially in the range between 80 and 95%.
